

July 30, 1957

G. F. NADEAU ET AL

2,801,191

REMOVABLE LAYERS FOR FILM

Filed Nov. 8, 1955

Fig. 1



Fig. 2



GALE F. NADEAU  
CRAYTON B. THOMPSON  
INVENTORS

BY *Daniel J. Mayne*  
*Harold N. Powell*

ATTORNEYS

# United States Patent Office

2,801,191

Patented July 30, 1957

1

2,801,191

## REMOVABLE LAYERS FOR FILM

Gale F. Nadeau and Crayton B. Thompson, Rochester, N. Y., assignors to Eastman Kodak Company, Rochester, N. Y., a corporation of New Jersey

Application November 8, 1955, Serial No. 545,644

10 Claims. (Cl. 117—138.8)

This invention relates to backed film or sheeting. More particularly this invention concerns photographic film carrying a new and improved backing.

As is well-known, film or sheeting quite frequently has backing or coating thereon. For example, photographic film is, in many instances, provided with a coating or layer on one or more of the surfaces, such as a layer or layers known as antihalation backings, antistatic layers and the like. These layers, which are provided for such purposes as aforementioned, in many instances for best performance should be relatively permanent for a period, such as during manufacturing operations, but should be capable of being removed.

For example, in the instance of photographic film it might be desired that the antistatic or antihalation backing remain on the film during manufacture and processing of the film. However, when a finished negative is produced it would be desired that such backings be eliminated.

Certain of the backings heretofore in use have presented problems either in difficulty of removal or in that special care has been required in the manufacture and handling of the film backed in accordance with practices prior to the present invention, so that the backing did not become removed prematurely.

It is apparent, therefore, that the development of a backing which not only satisfactorily performs the desired function such as performing as an antihalation backing, antistatic backing or the like, but which lends itself to removability at the proper time, represents a highly desirable result. We have found a material and its method of application to film and sheeting, as will be described in detail hereinafter, which constitutes an especially useful and improved backing on film and sheeting.

This invention has for one object to provide a film or sheet backed with a removable backing. Another object is to provide a photographic film carrying a new and improved removable backing. Still a further object is to provide a film or sheet carrying a backing which is relatively easily removable in a slightly acid media. Still another object is to provide a method of applying aminoacyl cellulose derivatives to photographic films as backings. Another object is to provide a method for the aforesaid whereby the aminoacyl derivative may contain various additives such as dyes, pigments and/or conducting agents. A particular object is to provide a photographic film of cellulose acetate with an aminoacyl cellulose derivative backing. Other objects will appear herein-after.

We have found that there are certain aminoacyl derivatives of cellulose which possess the unique quality of being soluble in slightly acid media. We have further found that these aminoacyl derivatives may be applied as coatings to films and sheets to provide various type layers and backings such as antihalation and antistatic backings, for example. These layers or coatings, because of the acid solubility as aforementioned, provide a backing that may be relatively readily removed as desired. That is, the backing may be removed by a slightly acid media such

2

as for example a 0.5% glacial acetic acid solution without damage to the film product.

For a more complete understanding of our invention reference is made to the attached drawing. In the drawing,

Fig. 1 is a diagrammatic, sectional view on an enlarged scale, generally illustrating a film product in accordance with the present invention.

Fig. 2 likewise is a diagrammatic, sectional view on an enlarged scale, illustrating a species of the film product of the present invention.

Specific examples of some of these aminoacyl cellulose derivatives which are useful in the present invention are as follows:

- 15 Cellulose acetate N,N-dimethylamino acetate  
Cellulose acetate N, N-diethylamino acetate  
Cellulose acetate N,N-dipropylamino acetate  
Cellulose acetate morpholino acetate  
Cellulose acetate butyrate N,N-diethylamino acetate  
20 Ethyl cellulose N,N-diethylamino acetate

In order to obtain aminoacylderivatives of the class indicated having the desired properties for backing purposes in accordance with the present invention, certain 25 procedures are preferably used in the preparation of such compounds. That is, the intermediate cellulose acetate chloroacetate used in the manufacture of the aminoacyl compounds preferably will have at least a 4% chlorine (halogen) content. On amination of the final aminoacyl 30 cellulose derivative will then have at least 1½% nitrogen.

The following description illustrates one method for the preparation of compounds such as may be employed in the present invention. It is to be understood, however, that while we prefer to use the CADA compounds prepared in accordance with the procedures which will be set forth, this is not to be regarded as a limitation on our invention. That is, CADA compounds, provided they have the desired composition and properties as above disclosed, even if prepared by other methods, would be within 40 the scope of the present invention.

In making the compounds used in the present invention, halogen-containing cellulose derivatives would be one of the starting materials. For example, halogen-containing cellulose derivatives such as cellulose acetate chloroacetates and ethylcellulose chloroacetates are illustrative. Other cellulose derivatives containing other acyl and chloroacetyl, chloropropionyl and the like may also comprise starting materials. As to methods for preparing halogen-containing cellulose derivatives, reference may be 50 made to the literature, i. e. Malm, Mench, Williams and Hiatt, Ind. Eng. Chem., 42, 1547 (1950).

The halogen-containing cellulose derivatives illustrated by cellulose chloroacetate in the dry condition and containing at least 4% of chlorine, is dissolved in a solvent 55 such as dioxane, acetone, methyl ethyl ketone, or other suitable solvent. There is then added at least two molar equivalents of a secondary amine based on the chlorine content of the cellulose derivative. This amount supplies one mole of amine to replace the chlorine atom and another mole to form amine hydrochloride which is insoluble in the reaction solvent and effectively removes the HCl liberated. This facilitates the forcing of the 60 amination reaction to completion and also prevents degradation of the cellulose ester by the liberated acid.

Secondary amines which may be used for the formation 65 of desirable dilute acid-soluble cellulose derivatives include dimethylamine, diethylamine, di-n-propylamine, di-isopropylamine, di-n-butylamine, morpholine, piperidine and the like. Mixed secondary aliphatic amines also may 70 be utilized in some instances. However, it should be noted that while the higher aliphatic secondary amines and the aromatic amines or the mixed aromatic-aliphatic



The resultant backed film product was separated into separate strips which were tested as just indicated. Here again the optical density was 1.5 and the resistivity less than  $1 \times 10^{10}$  ohms per sq. cm.

Another composition was made up using milled CADA which was free of any carbon, but was dissolved in an acetone-methanol solvent. Film base was coated therewith to give plain, unpigmented backing. This backing was tested for adherence and found to adhere satisfactorily even though the backed film base was subjected to various developing solutions and other types of photographic solutions.

#### Example II

In accordance with this example, 4% of the CADA material in this example was cellulose acetate N,N-diethylamino acetate) in a 75% acetone, 21% methanol solution, was applied to standard cellulose acetate film support. The solvent was evaporated to leave a thin backing by conventional procedure. This film support thus backed with the CADA was then immersed in a solution of the following composition:

2% nigrosine spirit jet (aniline black dye)  
1% aerosol AY (wetting agent of dicarboxylic acid ester 25  
type—American Cyanamid Co.)  
25% methanol  
72% ethanol

After suitably drying the dyed film to permit the evaporation of the methanol-ethanol solvent which had been used for the dye, there was obtained a film product having an excellent antihalation backing. Various test strips of this backed film product with the instant antihalation backing were subjected to different processing solutions and the backed film reexamined. In all instances it was found that the backing withstood the processing solutions and exhibited no tendency to peel from the film base. The test strips were then treated in a mild acetic acid solution with the result that the antihalation backing was readily removed leaving a clean film base surface.

In further runs under the present example, the nigrosine dye was replaced with an antistatic material known as Daxad 11 (polymerized sodium salts of alkyl aryl sulfonic acids—from Dewey and Almy Chemical Co.). It was found that this antistatic material was well carried in the CADA to provide a good antistatic backing on the film base.

In another run under this example,  $\beta$ -methacryloxyethylidemethyl ammonium methylsulfate was incorporated in the above-described CADA-acetone-methanol solution and standard cellulose acetate film base coated therewith. The resultant backing on the film not only adhered satisfactorily, but exhibited a surface resistivity less than  $1 \times 10^{10}$  ohms per sq. cm.

In another run under this example, butyl amine salt of cellulose acetate sulfate was incorporated in the above-described CADA-acetone-methanol solution and standard cellulose acetate film base coated therewith. The resultant backing on the film not only adhered satisfactorily, but exhibited a surface resistivity less than  $1 \times 10^{10}$  ohms per sq. cm.

In a further run under this example the backings containing additives Daxad 11,  $\beta$ -methacryloxyethylidemethyl ammonium methylsulfate, and butyl amine salt of cellulose acetate sulfate, just mentioned, were immersed in the above-described nigrosine dye solution. In each case this resulted in a backed film performing a dual function. That is, the backed film not only exhibited antihalation properties, but also exhibited antistatic properties. This backed film exhibiting these dual properties was then tested in various processing solutions and the adherence of the backing inspected. In all instances the backing withstood the processing solutions without indication of separation. However, the back-

ings were readily removable in a weak acetic acid solution.

#### Example III

In accordance with this example the coating applied to film base had the following formula:

1.7% nigrosine spirit jet  
2.1%  $\beta$ -methacryloxyethylidemethyl ammonium methylsulfate  
10 1.9% CADA (cellulose acetate N,N-diethylamino acetate  
0.3% aerosol AY  
77.0% acetone  
17.0% methanol

The layer dispersed on film base in this example was between 1.2 and 12.0 microns in thickness. The resultant backed film not only exhibited good antihalation protection but likewise measured a resistivity of less than  $1 \times 10^{10}$  ohms per sq. cm., thereby exhibiting satisfactory antistatic performance. Tests of the type referred to in the preceding examples indicated satisfactory adherence of this backing in various photographic processing solutions as well as removability in a weak acid solution.

#### Example IV

In accordance with this example, a standard roll of cellulose acetate film base was first backed with a backing solution of 1% butyl amine salt of cellulose acetate sulfate, 1% sodium acetate from a 70% acetone, 28% methanol solvent. In other words the film base was first backed by conventional procedure with backing which has heretofore been used in the art.

This first backing was then overcoated with a backing in accordance with the present invention. That is, the first-mentioned layer was then overcoated with a coating deposited from the following formula:

2% CADA (cellulose acetate N,N-diethylamino acetate);  
75% acetone  
23% methanol

The finished product was measured for surface resistivity and a value of less than  $.2 \times 10^{10}$  ohms per sq. cm. obtained, which was regarded as quite satisfactory particularly in the light of the additional advantages that were obtained. It was found that the second coat (overcoat) in accordance with the present invention quite effectively prevented softening of the first coat in high humidity and other such conditions which prevail in manufacturing operations such as emulsion coating. That is, the overcoat in accordance with the present invention permitted successful and practical utilization of the use of a first coat as above described under conditions where problems of adherence would arise in the event the overcoat in accordance with the present invention had not been employed.

Other runs in accordance with this example where the CADA coating is used as an overcoating were made. That is, runs were made where the overcoat was applied over a sensitometrically active backing. It was found that the overcoat in accordance with the present invention not only adhered satisfactorily, but prevented fogging of the emulsion when it was rolled against a backing that was sensitometrically active.

It can be seen from the foregoing examples that we have provided a new coating or backing material which may be utilized in various manners. That is, it may be used as a coating per se. This coating may be subsequently dyed or otherwise treated in several ways. Or, CADA coating may be used as a vehicle for various antistatic and dye materials. Also, our coating may be used as an overcoating on various coatings to protect such coatings so that the dual coated film product may be subjected to various manufacturing and processing operations.

While in the above examples we have referred to the application of our new CADA backing to cellulose acetate film base, which film base in general had either a

42-44% acetyl or an acetyl from between 34-42%, our invention is not limited to the use of such film base. In a manner similar to the treatment of cellulose acetate base we may likewise treat film or sheeting comprised of cellulose acetate propionate or cellulose acetate butyrate. We have found that solutions of CADA in solvents such as halogenated hydrocarbons or phenols may in a comparable manner be applied to sheeting made from polyesters such as polyethylene terephthalate. CADA may also be applied from methyl Cellosolve and methanol or 40% ethylene chloride and 60% methanol or 50% acetone and 50% methanol to polystyrene or Vinylite sheeting.

While in the above examples we have referred to the use of a nigrosine dye as this is a type of dye used quite frequently in the art, our new CADA backing may likewise be used with various other dyes such as acetate dyes (azo or anthraquinone) or fugitive dyes such as triphenylmethane or oxanole dyes.

Likewise in the above description, although we have referred to the use of mild acetic acid solution for removing the backing, since this is readily available and a very satisfactory type of acid to use for such purposes, our invention is not limited to this acid. Various other acid solutions, of which the following are illustrative, may be used as the acid media for removing the backing in accordance with the present invention: very dilute (0.01 to 0.10% of concentrated acid in water) solutions of mineral acids; hydrochloric, sulfuric or phosphoric.

While we have described the use of ketones, halogenated hydrocarbons and alcohols as solvents for preparing coating solutions of CADA, and these are preferred, other solvent combinations such as the following may be used; methyl Cellosolve, ethyl Cellosolve, and esters such as ethyl acetate and methyl Cellosolve acetate.

Likewise, where we have described the use of surface active agents such as aerscol AY, other agents such as Nacconol N, Arctic Syntex T or Padasol may be used. For example, according to the "Handbook of Material Trade Names," Zimmerman and Lavine, Nacconol N is a sodium alkyl aryl sulfonate (Allied Chemical & Dye Corp.), and Arctic Syntex T is a fatty acid amide sulfonate (Colgate-Palmolive Peet Company).

Therefore, it is apparent from the foregoing that we have provided a backed film or sheet which exhibits a number of improved properties and in which a certain latitude of modifications is possible.

We claim:

1. As a new product a thin plastic sheet principally comprised of a plastic from the group consisting of cellulose esters, polyesters, polystyrene and polyvinyl compounds carrying a layer at least on one surface thereof, which layer contains as the essential and principal component, a chemical compound illustrated by the following general formula:



2. As a new product, a thin plastic sheet principally comprised of a plastic from the group consisting of cellulose esters, polyesters, polystyrene and polyvinyl compounds carrying a layer at least on one surface thereof, which layer contains as the essential and principal component, a chemical compound illustrated as follows:



3. As an article of manufacture, a thin cellulose acetate sheet carrying at least on one surface thereof a thinner layer of a coating deposited from a solution of cellulose acetate N,N-dialkylamino acetate in a solvent therefor, said 5 first-mentioned coating having been treated with a solution comprising a dicarboxylic acid ester wetting agent and nigrosine spirit jet dye dissolved in a methanol-ethanol solvent.

4. As an article of manufacture, a thin cellulose acetate sheet carrying at least on one surface thereof a thinner layer of a coating deposited from a solution of an amino acyl derivative of cellulose from the group consisting of cellulose acetate N,N-diethylamino acetate, cellulose acetate N,N-dipropylamino acetate, cellulose acetate morpholino acetate, cellulose acetate butyrate N,N-diethylamino acetate, and ethyl cellulose N,N-diethylamino acetate, and carbon black in ethylene chloride and methanol solvents.

5. As an article of manufacture, a thin cellulose acetate sheet carrying at least on one surface thereof a thinner layer of a coating principally comprised of an aminoacyl derivative of cellulose from the group consisting of cellulose acetate N,N-dimethylamino acetate, cellulose acetate N,N-diethylamino acetate, cellulose acetate N,N-dipropylamino acetate, cellulose acetate morpholino acetate, cellulose acetate butyrate N,N-diethylamino acetate, and ethyl cellulose N,N-diethylamino acetate, but also containing a content of a polymerized sodium salt of alkyl aryl sulfonic acid.

6. As an article of manufacture, a thin cellulose acetate sheet carrying at least on one surface thereof a thinner layer of a coating principally comprised of an aminoacyl derivative of cellulose from the group consisting of cellulose acetate N,N-dimethylamino acetate, cellulose acetate N,N-diethylamino acetate, cellulose acetate N,N-dipropylamino acetate, cellulose acetate morpholino acetate, cellulose acetate butyrate N,N-diethylamino acetate, and ethyl cellulose N,N-diethylamino acetate but also containing a content of  $\beta$ -methacryloxyethylidemethyl ammonium methylsulfate.

7. The method of manufacturing film product which possesses antihalation and antistatic properties, which comprises obtaining a film base material, applying to at least one surface of said film base a composition made up of aminoacyl derivative of cellulose from the group consisting of cellulose acetate N,N-dimethylamino acetate, cellulose acetate N,N-diethylamino acetate, cellulose acetate N,N-dipropylamino acetate, cellulose acetate morpholino acetate, cellulose acetate butyrate N,N-diethylamino acetate, and ethyl cellulose N,N-diethylamino acetate, and antihalation dye, an antistatic material and solvent which will substantially dissolve the aforementioned ingredients and attack the film base to a limited extent, and evaporating off said solvent to leave a coating of the first-mentioned ingredients.

8. The method of manufacturing film product which possesses antihalation and antistatic properties comprising obtaining film base material, applying to at least one surface of said film base material a composition made up of aminoacyl derivative of cellulose from the group consisting of cellulose acetate N,N-dimethylamino acetate, cellulose acetate N,N-diethylamino acetate, cellulose acetate N,N-dipropylamino acetate, cellulose acetate morpholino acetate, cellulose acetate butyrate, N,N-diethylamino acetate, and ethyl cellulose N,N-diethylamino acetate, nigrosine spirit jet, polymerized sodium salt of alkyl aryl sulfonic acid, and solvent which will substantially dissolve the aforementioned ingredients and attack the film base to some extent, and evaporating off said solvent to leave a coating of the first-mentioned ingredients.

9. The method of manufacturing a film product which comprises obtaining cellulose acetate film base material

and applying to at least one surface of said film material a composition made up of cellulose acetate N,N-dialkylamino acetate, an antihalation dye, an antistatic material and solvent which will substantially dissolve the aforementioned ingredients and cause them to attach to the film base, and evaporating off said solvent to leave a coating of the first-mentioned ingredients.

10. As an article of manufacture, a cellulose ester film base carrying on at least one surface a layer which is thinner than the thickness of said film base, said layer being principally comprised of a compound from the group consisting of cellulose acetate N,N-dimethylamino acetate, cellulose acetate N,N-diethylamino acetate, cel-

lulose acetate N,N-dipropylamino acetate, cellulose acetate morpholino acetate, cellulose acetate butyrate N,N-diethylamino acetate, and ethyl cellulose N,N-diethylamino acetate, and said layer also having incorporated therein a content of carbon particles.

## References Cited in the file of this patent

## UNITED STATES PATENTS

10 2,072,870 Dreyfus ----- Mar. 9, 1937

## FOREIGN PATENTS

713,386 Great Britain ----- Aug. 11, 1954